

# UNITED STATES PATENT OFFICE.

FOSTER MILLIKEN, OF LAWRENCE, NEW YORK, ASSIGNOR TO FOSTER MILLIKEN,  
S. FULLERTON WEAVER, AND JAMES M. BEPPLIER, AS TRUSTEES.

## ALLOY.

1,354,989.

Specification of Letters Patent.

Patented Oct. 5, 1920.

No Drawing.

Application filed October 8, 1919. Serial No. 329,187.

*To all whom it may concern:*

Be it known that I, FOSTER MILLIKEN, a citizen of the United States, and a resident of Lawrence, in the county of Nassau and State of New York, have invented a new and Improved Alloy, of which the following is a full, clear, and exact description.

The object of the invention is to provide a new and improved alloy more especially designed for the manufacture of hose connections, valves, fittings and similar articles, and particularly such as are used in handling gasoline and lighter distillates of petroleum.

Another object is to provide an alloy not liable to cut or "wire draw."

The alloy consists of the following metals in about the following proportions, namely:

|    |        |          |           |
|----|--------|----------|-----------|
| 20 | Lead   | 10 to 14 | per cent. |
|    | Copper | 55 to 65 | " "       |
|    | Nickel | 6 to 11  | " "       |
|    | Zinc   | 14 to 18 | " "       |

These metals are melted together, and the resultant alloy is particularly well adapted to be cast into the various articles above referred to. The high percentage of the lead renders the alloy particularly useful for pressure work.

30

I claim:

An alloy consisting of the following metals in approximately the following proportions, namely: lead 10 to 14 per cent., copper 55 to 65 per cent., nickel 6 to 11 per cent., and zinc 14 to 18 per cent.

FOSTER MILLIKEN.